



US010188142B2

(12) **United States Patent**  
Fournier et al.

(10) **Patent No.:** US 10,188,142 B2  
(45) **Date of Patent:** Jan. 29, 2019

(54) **AMPHIPHILE-MODIFIED SORBENTS IN SMOKING ARTICLES AND FILTERS**

(71) Applicant: **Philip Morris USA Inc.**, Richmond, VA (US)

(72) Inventors: **Jay A. Fournier**, Richmond, VA (US); **Luan Zhaohua**, Midlothian, VA (US)

(73) Assignee: **Philip Morris USA Inc.**, Richmond, VA (US)

(\*) Notice: Subject to any disclaimer, the term of this patent is extended or adjusted under 35 U.S.C. 154(b) by 601 days.

(21) Appl. No.: **14/982,875**

(22) Filed: **Dec. 29, 2015**

(65) **Prior Publication Data**

US 2016/0128380 A1 May 12, 2016

**Related U.S. Application Data**

(62) Division of application No. 12/896,463, filed on Oct. 1, 2010, now Pat. No. 9,232,821, which is a division of application No. 10/740,510, filed on Dec. 22, 2003, now Pat. No. 7,827,996.

(51) **Int. Cl.**

*A24D 3/12* (2006.01)  
*A24D 3/14* (2006.01)  
*A24D 3/16* (2006.01)  
*A24D 3/06* (2006.01)  
*A24D 3/08* (2006.01)  
*A24D 3/10* (2006.01)

(52) **U.S. Cl.**

CPC ..... *A24D 3/12* (2013.01); *A24D 3/062* (2013.01); *A24D 3/067* (2013.01); *A24D 3/08* (2013.01); *A24D 3/10* (2013.01); *A24D 3/14* (2013.01); *A24D 3/166* (2013.01)

(58) **Field of Classification Search**

None

See application file for complete search history.

(56) **References Cited**

**U.S. PATENT DOCUMENTS**

2,695,618 A 11/1954 Policansky  
2,882,243 A 4/1959 Milton  
3,025,233 A 3/1962 Figert  
(Continued)

**FOREIGN PATENT DOCUMENTS**

DE 1038015 9/1958  
DE 2917313 A 11/1980

**OTHER PUBLICATIONS**

"Cationic Surfactant", <http://www.orica.com.au/Business%5...>  
CE75A4A2567D002000D6?OpenDocument, printed Aug. 7, 2001.  
(Continued)

*Primary Examiner* — Michael J Felton

(74) *Attorney, Agent, or Firm* — Buchanan Ingersoll & Rooney LLC

(57) **ABSTRACT**

Smoking articles which involve the use of amphiphile-modified sorbents are disclosed. The amphiphile-modified sorbent has at least one amphiphilic compound bound to an inorganic molecular sieve substrate. The amphiphile-modified sorbent selectively removes certain constituents from cigarette smoke, while maintaining other constituents, such as those that contribute to flavor. Methods for making cigarette filters and smoking articles using amphiphile-modified sorbents, as well as methods for smoking a cigarette containing an amphiphile-modified sorbent, are also provided.

**16 Claims, 3 Drawing Sheets**



(56)

## References Cited

## U.S. PATENT DOCUMENTS

|                 |         |                     |
|-----------------|---------|---------------------|
| 3,055,654 A     | 9/1962  | Harrison et al.     |
| 3,091,550 A     | 5/1963  | Doying              |
| 3,130,007 A     | 4/1964  | Breck               |
| 3,217,715 A     | 11/1965 | Berger et al.       |
| 3,247,195 A     | 4/1966  | Kerr                |
| 3,292,636 A     | 12/1966 | Mays                |
| 3,308,069 A     | 3/1967  | Wadlinger et al.    |
| 3,314,752 A     | 4/1967  | Kerr                |
| 3,327,718 A     | 6/1967  | Kilburn             |
| 3,572,348 A     | 3/1971  | Norman et al.       |
| 3,652,461 A     | 3/1972  | Dalton              |
| 3,702,886 A     | 11/1972 | Argauer et al.      |
| 3,703,901 A     | 11/1972 | Norman et al.       |
| 3,978,869 A     | 9/1976  | Uehara et al.       |
| 4,022,223 A     | 5/1977  | Rainer et al.       |
| 4,062,368 A     | 12/1977 | Crellin et al.      |
| 4,148,864 A     | 4/1979  | Groth et al.        |
| 4,177,822 A     | 12/1979 | Bryant, Jr. et al.  |
| 4,236,533 A     | 12/1980 | De Clara            |
| 4,246,009 A     | 1/1981  | Sawada et al.       |
| 4,246,910 A     | 1/1981  | Rainer et al.       |
| 4,252,687 A     | 2/1981  | Dale et al.         |
| 4,256,609 A     | 3/1981  | Dale et al.         |
| 4,317,460 A     | 3/1982  | Dale et al.         |
| 4,364,403 A     | 12/1982 | Horsewell et al.    |
| 4,397,321 A     | 8/1983  | Stuetz              |
| 4,454,056 A     | 6/1984  | Kittelmann et al.   |
| 4,604,110 A     | 8/1986  | Frazier             |
| 4,662,384 A     | 5/1987  | Green               |
| 4,964,426 A     | 10/1990 | Lee et al.          |
| 4,982,000 A     | 1/1991  | Earl et al.         |
| 5,060,672 A     | 10/1991 | Irimi et al.        |
| 5,098,684 A     | 3/1992  | Kresge et al.       |
| 5,102,643 A     | 4/1992  | Kresge et al.       |
| 5,108,725 A     | 4/1992  | Beck et al.         |
| 5,120,692 A     | 6/1992  | Beck                |
| 5,149,435 A     | 9/1992  | Laube               |
| 5,150,723 A     | 9/1992  | Lee et al.          |
| 5,204,376 A     | 4/1993  | Henmi et al.        |
| 5,212,131 A     | 5/1993  | Belding             |
| 5,258,340 A     | 11/1993 | Augustine et al.    |
| 5,261,948 A     | 11/1993 | Foley et al.        |
| 5,278,112 A     | 1/1994  | Klatte              |
| 5,360,023 A     | 11/1994 | Blakley et al.      |
| 5,370,785 A     | 12/1994 | Beck et al.         |
| 5,376,348 A     | 12/1994 | Stoilov et al.      |
| 5,396,909 A     | 3/1995  | Gentry et al.       |
| 5,404,890 A     | 4/1995  | Gentry et al.       |
| 5,482,915 A     | 1/1996  | Golden et al.       |
| 5,499,636 A     | 3/1996  | Baggett, Jr. et al. |
| 5,540,759 A     | 7/1996  | Golden et al.       |
| 5,568,819 A     | 10/1996 | Gentry et al.       |
| 5,657,772 A     | 8/1997  | Duke et al.         |
| 5,666,976 A     | 9/1997  | Adams et al.        |
| 5,692,525 A     | 12/1997 | Counts et al.       |
| 5,692,526 A     | 12/1997 | Adams et al.        |
| 5,705,269 A     | 1/1998  | Pimenov et al.      |
| 5,727,573 A     | 3/1998  | Meier et al.        |
| 5,738,793 A     | 4/1998  | Janks et al.        |
| 5,833,739 A     | 11/1998 | Klatte et al.       |
| 5,915,387 A     | 6/1999  | Baggett, Jr. et al. |
| 5,972,079 A     | 10/1999 | Foley et al.        |
| 5,985,790 A     | 11/1999 | Moskovitz et al.    |
| 5,988,176 A     | 11/1999 | Baggett, Jr. et al. |
| 6,026,820 A     | 2/2000  | Baggett, Jr. et al. |
| 6,074,974 A     | 6/2000  | Lee et al.          |
| 6,117,810 A     | 9/2000  | Lee et al.          |
| 6,119,699 A     | 9/2000  | Sung                |
| 6,168,773 B1    | 1/2001  | Sharp               |
| 6,209,547 B1    | 4/2001  | Koller et al.       |
| 6,261,986 B1    | 7/2001  | Bowman et al.       |
| 6,584,979 B2    | 7/2003  | Xue et al.          |
| 6,596,909 B2    | 7/2003  | Nishijima et al.    |
| 2001/0012820 A1 | 8/2001  | Nishijima et al.    |
| 2004/0016436 A1 | 1/2004  | Thomas              |

2004/0194792 A1 10/2004 Zhuang et al.  
 2005/0133047 A1 6/2005 Fournier et al.  
 2005/0133051 A1 6/2005 Luan et al.

## OTHER PUBLICATIONS

“Surfactant-Modified Zeolite (SMZ)—A Versatile, Inexpensive Sorbent for Removing Contaminants from Water”, <http://www.ees.nmt.edu/Hydro/faculty/Bowman/Research/zeopage/smz.html>, printed Jul. 31, 2001.

Zhaohui Li et al., Sorption of Ionizable Organic Solutes by Surfactant-Modified Zeolite, *Environ. Sci. Technol.* 2000, vol. 34, pp. 3756-3760.

Zhaohui Li et al., “Enhanced Reduction of Chromate and PCE by Pelletized Surfactant-Modified Zeolite/Zerovalent Iron”, *Environ. Sci. Technol.* 1999, vol. 33, pp. 4326-4330.

Zhaohui Li et al., “Counterion Effects on the Sorption of Cationic Surfactant and Chromate on Natural Clinoptilolite”, *Environ. Sci. technol.* 1997, vol. 31, pp. 2407-2412.

Gaydardjief S., et al., “Adsorption of Oxyanions with Surface Modified Zeolites”, *Acta Metallurgica Slovaca*, 4, Special Issue Apr. 2001, pp. 51-57.

Robert S. Bowman, “Surfactant-Altered Zeolites as Permeable Barriers for In Situ Treatment of Contaminated Groundwater”, Department of EARTH and Environmental Sciences, New Mexico Tech.

Robert S. Bowman, “SMZ + Microorganisms for Combined Sorption/ Biodegradation”, <http://www.ees.nmt.edu/bowman/research/SMZ/SMZBiodegrad.html>, printed Aug. 12, 2002.

Robert S. Bowman, “SMZ/ZVI Permeable Barrier Pilot Test”, <http://www.ees.nmt.edu/bowman/research/SMZ/SMZZVIPilotTest.html>, printed Aug. 12, 2002.

Robert S. Bowman, “SMZ for Removal of Pathogens from Sewage”, <http://www.ees.nmt.edu/bowman/research/SMZ/Pathogens.html>, printed Aug. 12, 2002.

Robert S. Bowman, “SMZ/ZVI Pellets for Combined Sorption/ Reduction”, <http://www.ees.nmt.edu/bowman/research/SMZ/SMZZVIProp.html>, printed Aug. 12, 2002.

Robert S. Bowman, “SMZ for Treatment of Oil Field Wastewaters”, <http://www.ees.nmt.edu/bowman/research/SMZ/ProdWater.html>, printed Aug. 12, 2002.

Robert S. Bowman, “SMZ Permeable Barrier Test Facility”, <http://www.ees.nmt.edu/bowman/research/SMZ/PilotTestFacility.html>, printed Aug. 12, 2002.

Robert S. Bowman, “SMZ Permeable Barrier Test Results”, <http://www.ees.nmt.edu/bowman/research/SMZ/SMZPilotTest.html>, printed Aug. 12, 2002.

Robert S. Bowman, Mechanisms of Surfactant and Contaminant Sorption by SMZ, <http://www.ees.nmt.edu/bowman/research/SMZ/SMZSorpMech.html>, printed Aug. 12, 2002.

Robert S. Bowman, “Zeolite-Surfactant Interactions”, <http://www.ees.nmt.edu/bowman/research/SMZ/ZeoSurflnt.html>, printed Aug. 12, 2002.

Robert S. Bowman, “Surfactant-Modified-Zeolites (SMA) and their Applications to Environmental Remediation”, <http://www.ees.nmt.edu/bowman/research/SMZ/>, printed Aug. 12, 2002.

Robert S. Bowman, “Properties of Zeolites”, <http://www.ees.nmt.edu/bowman/research/SMZ/ZeoProp.html>, printed Aug. 12, 2002.

Robert S. Bowman, “Sorption of Anions, Cations, and Neutral Organics by SMA”, <http://www.ees.nmt.edu/bowman/research/SMZ/SMZSorp.html>, printed Aug. 12, 2002.

March, “Advanced Organic Chemistry”, (John Wiley & Sons Inc., 1995) (reference provided upon request).

House, “Modern Synthetic Reactions” (Benjamin Cummings, 1972) (reference provided upon request).

Robb, I.D., Ed., “Specialist Surfactants”, Blackie Academic and Professional, First Edition, 1997, pp. 9-10.

Shiverick, K. T. et al., “Cigarette Smoking and Pregnancy: Ovarian, Uterine and Placental Effects”, *Placenta*, vol. 20, Issue 4, May 1999, pp. 265-272, ISSN 0143-4004, DOI: 10.1053/plac.1998.0377 (<http://www.sciencedirect.com/science/article/B6WPD-45CRJY-1P/2/06f14ded037185c4659fc1b92544b3>).



FIG. 1



FIG. 2



FIG. 3



FIG. 4



FIG. 5



FIG. 6



FIG. 7



FIG. 8

# AMPHIPHILE-MODIFIED SORBENTS IN SMOKING ARTICLES AND FILTERS

## CROSS-REFERENCE TO RELATED APPLICATIONS

This application is a divisional application of U.S. application Ser. No. 12/896,463, filed on Oct. 1, 2010, which is a divisional application of U.S. application Ser. No. 10/740,510, filed on Dec. 22, 2003, the entire contents of each of which is hereby incorporated by reference.

## BACKGROUND

Certain filter materials have been suggested for incorporation into cigarette filters, including cotton, paper, cellulose, and certain synthetic fibers. However, such filter materials generally only remove particulate and condensable components from tobacco smoke. Thus, they are usually not optimal for the removal of certain gaseous components from tobacco smoke, e.g., volatile organic compounds.

## SUMMARY

Amphiphile-modified sorbents for removing one or more selected constituents from mainstream smoke are provided. In an embodiment, one or more constituents can be selectively removed from mainstream tobacco smoke, while retaining other constituents, such as those relating to flavor.

The selected constituent of mainstream smoke may be removed by the amphiphile-modified sorbent through molecular sieving, ion exchange, hydrophobic interactions, chelation, and/or chemical binding. Preferably, the selected constituent of mainstream smoke that is removed may be at least one of a hydrocarbon, polar organic and/or organic compound. Preferably, the selected constituent of mainstream smoke that is removed is an aldehyde, carbon monoxide, 1,3-butadiene, isoprene, acrolein, acrylonitrile, hydrogen cyanide, o-toluidine, 2-naphthylamine, nitrogen oxide, benzene, N-nitrosonornicotine, phenol, catechol, benz(a)anthracene, and/or benzo(a)pyrene. More preferably, the constituent is an aldehyde.

In an embodiment, a smoking article is provided, which comprises an amphiphile-modified sorbent having at least one amphiphilic compound bound to an inorganic molecular sieve substrate. Examples of smoking articles include, but are not limited to a cigarette, a pipe, a cigar and a non-traditional cigarette. Preferably, the smoking article is a cigarette. Preferably, the smoking article is a cigarette including from about 50 mg to about 300 mg of the amphiphile-modified sorbent, more preferably from about 100 mg to about 200 mg of the amphiphile-modified sorbent. Preferably, the amphiphile-modified sorbent is located in a filter of the smoking article.

In yet another embodiment, a cigarette filter is provided, which comprises an amphiphile-modified sorbent having at least one amphiphilic compound bound to an inorganic molecular sieve substrate. Examples of filters include but are not limited to a mono filter, a dual filter, a triple filter, a cavity filter, a recessed filter or a free-flow filter. Preferably, the amphiphile-modified sorbent of the cigarette filter removes at least some of at least one selected constituent of mainstream smoke, more preferably removes at least some of a hydrocarbon or a polar organic compound constituent from mainstream smoke, and most preferably removes at least some of an aldehyde constituent from mainstream smoke.

The filter preferably comprises at least one material selected from the group consisting of cellulose acetate tow, cellulose paper, mono cellulose, mono acetate, and combinations thereof. In an embodiment, the amphiphile-modified sorbent is incorporated into one or more cigarette filter parts selected from the group consisting of shaped paper insert, a plug, a space, cigarette filter paper, and a free-flow sleeve.

Preferably, the amphiphile-modified sorbent is incorporated with cellulose acetate fibers forming a plug or a free-flow filter element, or incorporated with polypropylene fibers forming a plug or free-flow filter element. The amphiphile-modified sorbent may also be incorporated in at least one of a mouthpiece filter plug, a first tubular filter element adjacent to the mouthpiece filter plug, and a second tubular filter element adjacent to the first tubular element. In yet another embodiment, the amphiphile-modified sorbent is incorporated in at least one part of a three-piece filter including a mouthpiece filter plug, a first filter plug adjacent to the mouthpiece filter plug, and a second filter plug adjacent to the first filter plug.

In another embodiment, a method of making a cigarette filter is provided, which comprises incorporating an amphiphile-modified sorbent having at least one amphiphilic compound bound to an inorganic molecular sieve substrate into a cigarette filter.

In yet another embodiment, a method of making a cigarette is provided, which comprises: (i) providing a cut filler to a cigarette making machine to form a tobacco column; (ii) placing a paper wrapper around the tobacco column to form a tobacco rod; (iii) providing a cigarette filter comprising an amphiphile-modified sorbent having at least one amphiphilic compound bound to an inorganic molecular sieve substrate; and (iv) attaching the cigarette filter to the tobacco rod to form the cigarette.

In an embodiment, a method of smoking a cigarette is provided, which comprises lighting the cigarette to form smoke and drawing the smoke through the cigarette, wherein during the smoking of the cigarette, the amphiphile-modified sorbent removes one or more selected constituents from mainstream smoke.

Preferably, the amphiphilic compound may be covalently bound to the surface of the molecular sieve, or electrostatically bound to the surface of the molecular sieve.

Preferably, the amphiphile-modified sorbent is in particle form having an average mesh size from about 20 mesh to about 60 mesh.

Preferably, the amphiphilic compound comprises from about 4 to about 24 carbons, more preferably from about 6 to about 18 carbons. Preferably, the amphiphilic compound is an alkyl silane comprising an alkyl group having four or more linearly connected carbon atoms. Preferably, the amphiphilic compound is an alkyl quaternary ammonium cation or an alkyl silane.

Examples of inorganic molecular sieve substrates include, but are not limited to, the group consisting of zeolite, aluminophosphate, mesoporous silicate, mesoporous aluminosilicate, and mixtures thereof. Preferably, the inorganic molecular sieve substrate is a zeolite selected from the group consisting of zeolite ZSM-5, zeolite A, zeolite X, zeolite Y, zeolite K-G, zeolite ZK-5, zeolite Beta, zeolite ZK-4, and mixtures thereof, and more preferably the zeolite is selected from the group consisting of zeolite A, zeolite ZSM-5, zeolite X, and mixtures thereof.

## BRIEF DESCRIPTION OF THE DRAWINGS

FIG. 1 is a partially broken-away perspective view of a cigarette incorporating one embodiment wherein folded

paper containing amphiphile-modified sorbent is inserted into a hollow portion of a tubular filter element of the cigarette.

FIG. 2 is a partially broken-away perspective view of another embodiment wherein amphiphile-modified sorbent is incorporated in folded paper and inserted into a hollow portion of a first free-flow sleeve of a tubular filter element next to a second free-flow sleeve.

FIG. 3 is a partially broken-away perspective view of another embodiment wherein amphiphile-modified sorbent is incorporated in a plug-space-plug filter element.

FIG. 4 is a partially broken-away perspective view of another embodiment wherein amphiphile-modified sorbent is incorporated in a three-piece filter element having three plugs.

FIG. 5 is a partially broken-away perspective view of another embodiment wherein amphiphile-modified sorbent is incorporated in a four-piece filter element having a plug-space-plug arrangement and a hollow sleeve.

FIG. 6 is a partially broken-away perspective view of another embodiment wherein amphiphile-modified sorbent is incorporated in a three-part filter element having two plugs and a hollow sleeve.

FIG. 7 is a partially broken-away perspective view of another embodiment wherein amphiphile-modified sorbent is incorporated in a two-part filter element having two plugs.

FIG. 8 is a partially broken-away perspective view of another embodiment wherein amphiphile-modified sorbent is incorporated in a filter element which may be used in a smoking article.

#### DETAILED DESCRIPTION OF PREFERRED EMBODIMENTS

The amphiphile-modified sorbents described below can be used, for example, in smoking articles for selective removal of one or more selected constituents of mainstream smoke. By "selective removal" is meant that certain constituents are at least partially removed from mainstream smoke, while other constituents are not substantially removed. The term "selective" also encompasses preferential removal of certain constituents from mainstream smoke, i.e. where more than one constituent may be removed, but where one constituent is removed to a greater extent than another constituent.

With reference to a cigarette, the term "mainstream" smoke refers to the mixture of gases passing down the tobacco rod and issuing through the filter end, i.e. the amount of smoke issuing or drawn from the mouth end of a smoking article during smoking.

The term "molecular sieve" as used herein refers to an ordered porous material such as aluminosilicates, which are commonly called zeolites, or aluminophosphates, mesoporous silicates, and related porous materials such as various porous metal oxides, which may comprise further inorganic or organic ions and/or metals. A molecular sieve as used herein further refers to a material having pores with dimensions less than about 500 Å, preferably less than 300 Å, including microporous and mesoporous molecular sieves. The term "microporous molecular sieves" generally refers to such materials having pore sizes of about 20 Å or less, while the term "mesoporous molecular sieves" generally refers to such materials with pore sizes of about 20-500 Å and preferably 20 to 300 Å.

The term "sorption" denotes filtration through absorption and/or adsorption. Sorption is intended to cover interactions on the outer surface of the sorbent, as well as interactions

within the pores, such as channels or cavities, of the sorbent. In other words, a sorbent is a substance that has the ability to condense or hold molecules of other substances on its surface, and/or the ability to take up another substance, i.e. through penetration of the other substance into its inner structure or into its pores. The term adsorption also denotes filtration through physical sieving, i.e. capture of certain constituents in the pores of the sorbent. The term "sorbent" as used herein refers to either an adsorbent, an absorbent, or a substance that functions as both an adsorbent and an absorbent.

The terms "amphiphile" and "amphiphilic" as used herein refer to any substance comprising at least both a first portion (usually substantially non-polar) which, if separate from the amphiphile, would have a substantially greater solubility in, or a greater attraction to, an organic solvent, (i.e., acetonitrile, hexane, oil, and the like) than water, and a second portion (usually at least partially polar) which, if separate from the amphiphile, would be soluble in water or, if insoluble, may exist in a substantially hydrated form. The amphiphile itself may or may not be soluble in water or any particular, organic solvent. For example, compounds such as alkyl quaternary ammonium cations are considered amphiphiles because the molecules comprise a more hydrophobic alkyl segment and a more hydrophilic ammonium group. Likewise, an alkyl silane is considered an amphiphile because the molecules comprise a more hydrophobic alkyl segment and a more hydrophilic silane group. In another sense of the term, for example, an amphiphile-modified sorbent is also amphiphilic because the insoluble inorganic substrate particles may commonly be substantially hydrated by themselves while the hydrophobic portions (i.e. alkyl chains) of the amphiphilic coating are more soluble in oil than in water.

With respect to the amphiphile-modified sorbents, a naturally hydrophilic molecular sieve substrate is rendered more hydrophobic by one or more amphiphilic compounds. Preferably, the amphiphile coating can create a more hydrophobic exterior surface of the inorganic molecular sieve substrate without changing the nature of the interior micropores, thus providing multiple selective sorbent functionality. For instance, the surface of the amphiphile-modified sorbent may be rendered capable of retaining organic constituents of smoke, while the internal pores of the inorganic molecular sieve substrate may retain the ability to adsorb constituents of smoke that are smaller than the internal pores.

In one embodiment, the amphiphilic compounds may comprise specific functional groups in order to confer certain desired properties, such as electrostatic charge, ion exchange capacity, and reactive functional groups. Selected constituents of mainstream smoke may be specifically targeted and removed by a combination of molecular sieving, ion exchange, hydrophobic interactions, chelation, and/or covalent binding.

Preferably the amphiphile and sorbed smoke constituents are prevented from entering or re-entering the smoke stream because the amphiphile is either electrostatically or covalently bound to the inorganic molecular sieve substrate. In a preferred embodiment, properties of the amphiphile and inorganic molecular sieve substrate may be varied individually or in combination to target specific classes of gas-phase smoke constituents. For example, the hydrophobicity of the amphiphile may be adjusted to target certain classes of constituents, and/or reactive functional groups of the amphiphile may be chosen to react with certain classes of constituents. Moreover, the molecular sieve pore sizes may be chosen or modified to match specific constituents, and/or

catalytic constituents may be embedded within the molecular sieve to chemically react with specific constituents.

This aspect is advantageous over filter arrangements wherein gaseous constituents are non-selectively absorbed, adsorbed, or otherwise removed from a smoke stream. With an amphiphile coating the external surface of the molecular sieve, the surface chemistry is changed, which can lead to an increased capacity for the absorption of nonpolar organic compounds. Furthermore, the ion exchange capacity of the molecular sieve and the accessibility of polar molecules to the interior spaces of the molecular sieve and to catalytic sites which may be contained therein are maintained. By selecting the properties of the amphiphile, sequestration of specific hydrophobic constituents such as aromatic hydrocarbons may be optimized. By providing a specific functional group to the amphiphile, properties not inherent in inorganic molecular sieves may be incorporated into the filter arrangement. Examples include hydrophobicity, anion exchange, metal chelation, and specific reactivities. A preferred reactivity to aldehydes may be provided, for example, by primary amine groups which can covalently bind aldehydes. Anion exchange capacity may be provided to modified zeolites by positively charged functional substituents of the amphiphile. Metal chelation may be provided by including arrangements of acidic functional groups in a substituted alkyl chain of an amphiphile. For example, metal chelating groups may be covalently incorporated in some or all of the amphiphilic compounds coating the molecular sieve sorbent.

The inorganic molecular sieve substrate may be a zeolite. Zeolites are porous materials predominantly comprised of aluminosilicate. Zeolite pores may be more or less uniform micropores and may have pore dimensions over a range of sizes, e.g., below 20 Å; the material may further comprise additional metals and metal oxides. Synthetic zeolite materials may have more uniform pore dimensions and a more ordered structure. Various zeolite types are described, for example, in U.S. Pat. No. 3,702,886 (zeolite ZSM-5), U.S. Pat. No. 2,882,243 (zeolite A), U.S. Pat. No. 2,882,244 (zeolite X), U.S. Pat. No. 3,130,007 (zeolite Y), U.S. Pat. No. 3,055,654 (zeolite K-G), U.S. Pat. No. 3,247,195 (zeolite ZK-5), U.S. Pat. No. 3,308,069 (zeolite Beta), U.S. Pat. No. 3,314,752 (zeolite ZK-4). A source of natural zeolite in North America is the St. Cloud Mining Company, Truth or Consequences, N. Mex. One preferred characteristic for the zeolites is a well defined pore size. Preferred zeolite molecular sieve substrate materials include A, ZSM-5 and Y-type zeolites, or combinations thereof.

The surface of a preferred zeolite has a permanent negative charge. Therefore, when zeolite is used as the molecular sieve substrate, the amphiphile compounds may be any amphiphile compound possessing a cationic charge. Preferably, the cationic charge is a permanent charge. The interaction of the negatively charged surface and the positively charged amphiphile serves to stably bind the amphiphile to the substrate. The amphiphile may thus be retained on the zeolite surface without substantial loss during washing and processing steps of manufacturing and may be retained on the substrate under the conditions of intended use. Alternatively, silicate groups at the surface of zeolite may be utilized to covalently bind an alkyl silane amphiphile to the surface of a molecular sieve substrate. In this embodiment, the amphiphile is covalently bonded to the molecular sieve throughout processing and intended use and is therefore a preferred embodiment.

The inorganic molecular sieve substrate may be a mesoporous silicate, a mesoporous aluminosilicate, or a silica gel. Mesoporous silicates are described, for example, in

patents relating to MCM-41 and MCM-48 and SBA-15; such as U.S. Pat. Nos. 5,098,684, 5,102,643 and 5,108,725, which are all hereby incorporated by reference in their entirety. Silica gel materials and methods for making such materials, are described, for example, in U.S. Pat. Nos. 4,148,864, 5,376,348 and 6,168,773, which are all hereby incorporated by reference in their entirety.

Cationic amphiphiles may be electrostatically bound to a negatively charged molecular sieve such as a zeolite. Cationic amphiphiles exist as ions in solution and the cationic portion of the compound is surface active. Quaternary ammonium compounds may be regarded, as analogous to an ammonium chloride salt molecule in which all four hydrogen atoms are replaced by organic radicals. When one of these replacement radicals is a straight-chain, primary alkyl of about 6-18 carbon atoms chain length and the others are of about 1-3 carbon atoms, then the compound will be reasonably water soluble and surface active. If two or more of the substituent radicals are higher alkyls, then the compound retains its cationic nature but may become water-insoluble. For example, suitable quaternary ammonium cationic alkyl compounds include, but are not limited to, those with the general formula:



where n=0, 1 or 2, preferably 0;

N is a nitrogen atom;

R<sup>1</sup> is an aliphatic, saturated or unsaturated, straight, branched, or cyclic, substituted or unsubstituted chain of 1 to 24 carbons, preferably 6-18 carbons. Optionally, R<sup>1</sup> may be substituted, for example, at any number of positions with one or more of —H, —NH<sub>2</sub>, —OH, —SH, or —COOH. Optionally, R<sup>1</sup> may be interrupted, for example, by one or more of —NH—, —CH=CH—, —CHR<sup>1</sup>—, —CR<sup>1</sup>R<sup>1</sup>—, or —NR<sup>1</sup>—; where R<sup>1</sup> and R<sup>1</sup> are alkyl groups such as R<sup>1</sup> and may be the same or different. In general, R<sup>1</sup> may alternatively be any organic radical including carbohydrate or benzalkyl groups. In a preferred embodiment, R<sup>1</sup> is a straight aliphatic chain of about 3-24 carbon atoms, preferably 4-20 carbon atoms, more preferably 6-18 carbon atoms. R<sup>1</sup> may be optionally substituted at one or more positions, for example at a terminal position. Substituent groups may be chosen to convey a specific functionality to the amphiphile.

A primary amine group is useful for the specific removal of aldehydes. Carboxyl and/or sulfides may be chosen to chelate metals. A second same or different alkyl chain may replace one of the (CH<sub>3</sub>(CH<sub>2</sub>)<sub>n</sub>) groups. The amphiphile composition may comprise a single species or a mixture of amphiphile compounds. Various aliphatic chain lengths, degree and mode of unsaturation (cis and/or trans), branched and unbranched chains may be combined in mixtures in order to convey a desired spectrum of adsorptivity. Such compounds are widely available from a variety of manufacturers. The amphiphile compounds may be prepared using any suitable method; for example, see March, *Advanced Organic Chemistry* (John Wiley & Sons Inc., 1995); House, *Modern Synthetic Reactions* (Benjamin Cummings, 1972); or U.S. Pat. Nos. 4,982,000; 5,545,749 and the patents referenced therein. The amphiphile may also be any other cationic amphiphile. Acceptable alternatives which are commercially available or which may be made by well known synthetic methods include, for example, imidazolines, ethoxylated amines, and quaternary phospholipids.

In an embodiment, an amphiphile-modified molecular sieve sorbent may be made by combining an amphiphile compound in solution and a zeolite molecular sieve sub-

strate. The amphiphile may be in the form of a chloride salt in aqueous solution. Certain amphiphile compounds such as un-substituted alkyl quaternary ammonium cations can form bilayers on the substrate surface at sufficiently high concentrations. However, the outer-layer may be removed by repeated washing. Amphiphile concentrations below the critical micellar concentration may be used for formation of a monolayer of amphiphile on the exterior of a zeolite. The amphiphile is generally too large to enter the interior channels of a microporous molecular sieve (i.e., having a pore diameter of about 20 Å or less). After a period of time sufficient to allow cation exchange, the amphiphile-modified zeolite material is removed from the solution and may be washed with water. The amphiphile-modified zeolite material may be dried and incorporated into filter arrangements.

A preferred amphiphile-modified sorbent can be prepared as follows: Add about 10 grams of ZSM-5 zeolite powder to about 100 mL of a aqueous solution of cetyltrimethylammonium bromide (10% by weight) followed by stirring at room temperature for about 2 hours. The mixture is then transferred into a Teflon-lined pressure vessel and heated at about 150° C. for about 48 hours. The final solid product is filtered, washed with distilled water, and dried in air about 100° C. for about 12 hours. In this procedure the loading of the amphiphile is controlled by the concentration of the alkyl quaternary ammonium compound in the starting aqueous solution.

In an alternative embodiment, the amphiphile may be an alkyl silane. Examples include alkyl silane compounds such as those with the general formula:



where X may be for example a halogen such as Cl—, HO—,  $\text{CH}_3\text{O}$ —, or  $\text{CH}_3\text{CH}_2\text{O}$ —;

Si is a silicon atom;

$\text{R}^1$  is an aliphatic, saturated or unsaturated, straight, branched, or cyclic, substituted or unsubstituted chain of 3 to 24 carbons, preferably 4-20 carbons, more preferably 6-18 carbons. Optionally,  $\text{R}^1$  may be substituted, for example, at any number of positions with one or more of —H, —NH<sub>2</sub>, —OH, —SH or —COOH. Optionally,  $\text{R}^1$  may be interrupted, for example, by one or more of —NH—, —CH=CH—, —CHR<sup>1</sup>, —CR<sup>1</sup>R<sup>1</sup>— or —NR<sup>1</sup>—; where R<sup>1</sup> and R<sup>1</sup> are alkyl groups such as R<sup>1</sup> and may be the same or different. In general, R<sup>1</sup> may alternatively be any organic radical including carbohydrate or benzalkyl groups. In a preferred embodiment, R<sup>1</sup> is a straight aliphatic chain of about 3-24 carbon atoms, preferably 4-20 carbon atoms, more preferably 6-18 carbon atoms. R<sup>1</sup> may be optionally substituted at one or more positions, for example at a terminal position. Substituent groups may be chosen to convey a specific functionality to the amphiphile. A primary amine group is useful for the specific removal of aldehydes. Carboxyl and/or sulfides may be chosen to chelate metals. The amphiphile composition may comprise a single species or a mixture of amphiphile compounds. Various aliphatic chain lengths, degree and mode of unsaturation (cis and/or trans), branched and unbranched chains may be combined in mixtures in order to convey a desired spectrum of adsorptivity.

The amphiphile compounds may be prepared using any suitable technique. For routine synthetic methods see for example: March, *Advanced Organic Chemistry* (John Wiley & Sons Inc., 1995) and House, *Modern Synthetic Reactions* (Benjamin Cummings, 1972). In addition, a variety of

amphiphilic compounds are commercially available from a variety of manufacturers, such as Dow Corning and Union Carbide.

Thus, in an alternative embodiment, an alkyl silane amphiphile may be covalently bonded to the surface of a molecular sieve substrate material. A zeolite substrate may be prepared by drying at a temperature and pressure sufficient to remove essentially all bound water, for example at 100°-200° C. for 1 or 2 or more hours and optionally under 10 a reduced pressure and/or in an atmosphere of dry inert gas. An alkyl trichlorosilane may be dissolved in methanol which can result in the substitution of three methoxy groups bound to the silicon atom; a resulting alkyl trimethoxysilane may be distilled under conditions sufficient to remove substantially all of the liquid methanol and residual water without decomposing the alkyl methoxysilane composition. An alkyl methoxysilane composition and the molecular sieve may be combined in an organic solvent such as toluene, benzene, xylene, hexanes, cyclo-hexane, alcohols or other well 15 known solvents which may dissolve or suspend the alkyl silane. The organic solvent is preferably anhydrous and capable of dissolving the amphiphile. The suspension of molecular sieve particles such as zeolite and alkyl silane in organic solvent may be stirred and the temperature may be 20 maintained at an elevated temperature sufficient to allow the covalent reaction of the silane with the silica groups of the molecular sieve. The temperature is preferably at or lower than the boiling point of the anhydrous organic solvent. For example, the temperature of the mixture of molecular sieve 25 particles and alkyl silane in organic fluid may be maintained at 100° to 200° C. for 1 to 4 or more hours. The mixture may be maintained in an inert gas atmosphere such as dry nitrogen gas or argon. The amphiphile-modified sorbent may be separated from the solvent for example by filtration or 30 decanting. The amphiphile-modified sorbent may optionally be washed one or more times with one or more solvents such as water or alcohols. The amphiphile-modified sorbent may then be dried at an elevated temperature, for example about 100° C. for 1-8 hours or more.

Another preferred amphiphile-modified sorbent can be prepared as follows: Add about 10 grams of ZSM-5 zeolite powder to a solution containing about 100 mL of dry toluene and about 25 grams of octadecytrimethoxysilane followed by vigorous shaking or stirring at room temperature for 40 about 10 minutes. The suspension is then transferred into a Teflon-lined pressure vessel, sealed and heated at about 100° C. for about 12 hours. The final solid product is filtered, washed with about 100 mL of dry toluene followed by about 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 951

inserted into a hollow portion of the cigarette filter. The support is preferably in the form of a sheet material such as crepe paper, filter paper, or tipping paper. However, other suitable support materials such as organic or inorganic cigarette compatible materials can also be used.

FIG. 1 illustrates a cigarette 2 having a tobacco rod 4, a filter portion 6, and a mouthpiece filter plug 8. As shown, amphiphile-modified sorbent can be loaded onto folded paper 10 inserted into a hollow cavity such as the interior of a free-flow sleeve 12 forming part of the filter portion 6.

FIG. 2 shows a cigarette 2 having a tobacco rod 4 and a filter portion 6, wherein the folded paper 10 is located in the hollow cavity of a first free-flow sleeve 13 located between the mouthpiece filter 8 and a second free-flow sleeve 15. The paper 10 can be used in forms other than as a folded sheet. For instance, the paper 10 can be deployed as one or more individual strips, a wound roll, etc. In whichever form, a desired amount of amphiphile-modified sorbent can be provided in the cigarette filter portion by adjusting the amount of amphiphile-modified sorbent coated per unit area of the paper and/or the total area of coated paper employed in the filter (e.g., higher amounts of amphiphile-modified sorbent can be provided simply by using larger pieces of coated paper). In the cigarettes shown in FIGS. 1 and 2, the tobacco rod 4 and the filter portion 6 are joined together with tipping paper 14. In both cigarettes, the filter portion 6 may be held together by filter overwrap 11.

The amphiphile-modified sorbent can be incorporated into the filter paper in a number of ways. For example, the amphiphile-modified molecular sieve can be mixed with water to form a slurry. The slurry can then be coated onto pre-formed filter paper and allowed to dry. The filter paper can then be incorporated into the filter portion of a cigarette in the manner shown in FIGS. 1 and 2. Alternatively, the dried paper can be wrapped into a plug shape and inserted into a filter portion of the cigarette. For example, the paper can be wrapped into a plug shape and inserted as a plug into the interior of a free-flow filter element such as a polypropylene or cellulose acetate sleeve. In another arrangement, the paper can comprise an inner liner of such a free-flow filter element.

Alternatively, the amphiphile-modified molecular sieve is added to the filter paper during the paper-making process. For example, the amphiphile-modified molecular sieve can be mixed with bulk cellulose to form a cellulose pulp mixture. The mixture can be then formed into filter paper according to methods known in the art.

In another embodiment, the amphiphile-modified sorbent is incorporated into the fibrous material of the cigarette filter portion itself. Such filter materials include, but are not limited to, fibrous filter materials including paper, cellulose acetate fibers, and polypropylene fibers. This embodiment is illustrated in FIG. 3, which shows a cigarette 2 comprised of a tobacco rod 4 and a filter portion 6 in the form of a plug-space-plug filter having a mouthpiece filter 8, a plug 16, and a space 18. The plug 16 can comprise a tube or solid piece of material such as polypropylene or cellulose acetate fibers. The tobacco rod 4 and the filter portion 6 are joined together with tipping paper 14. The filter portion 6 may a filter overwrap 11. The filter overwrap 11 containing traditional fibrous filter material and amphiphile-modified sorbent can be incorporated in or on the filter overwrap 11 such as by being coated thereon. Alternatively, the amphiphile-modified sorbent can be incorporated in the mouthpiece filter 8, in the plug 16, and/or in the space 18. Moreover, the amphiphile-modified sorbent can be incorporated in any element of the filter portion of a cigarette. For example, the

filter portion may consist only of the mouthpiece filter 8 and the amphiphile-modified sorbent can be incorporated in the mouthpiece filter 8.

FIG. 4 shows a cigarette 2 comprised of a tobacco rod 4 and filter portion 6. This arrangement is similar to that of FIG. 3 except the space 18 is filled with granules of amphiphile-modified sorbent or a plug. 15 made of material such as fibrous polypropylene or cellulose acetate containing amphiphile-modified sorbent. As in the previous embodiment, the plug 16 can be hollow or solid and the tobacco rod 4 and filter portion 6 are joined together with tipping paper 14. There is also a filter overwrap 11.

FIG. 5 shows a cigarette 2 comprised of a tobacco rod 4 and a filter portion 6 wherein the filter portion 6 includes a mouthpiece filter 8, a filter overwrap 11, tipping paper 14 to join the tobacco rod 4 and filter portion 6, a space 18, a plug 16, and a hollow sleeve 20. The amphiphile-modified sorbent can be incorporated into one or more elements of the filter portion 6. For instance, the amphiphile-modified sorbent can be incorporated into the sleeve 20 or granules of the amphiphile-modified sorbent can be filled into the space within the sleeve 20. If desired, the plug 16 and sleeve 20 can be made of material such as fibrous polypropylene or cellulose acetate containing amphiphile-modified sorbent. As in the previous embodiment, the plug 16 can be hollow or solid.

FIGS. 6 and 7 show further modifications of the filter portion 6. In FIG. 6, cigarette 2 is comprised of a tobacco rod 4 and filter portion 6. The filter portion 6 includes a mouthpiece filter 8, a filter overwrap 11, a plug 22, and a sleeve 20, and the amphiphile-modified sorbent can be incorporated in one or more of these filter elements. In FIG. 7, the filter portion 6 includes a mouthpiece filter 8 and a plug 24, and the amphiphile-modified sorbent can be incorporated in one or more of these filter elements. Like the plug 16, the plugs 22 and 24 can be solid or hollow. In the cigarettes shown in FIGS. 6 and 7, the tobacco rod 4 and filter portion 6 are joined together by tipping paper 14.

Various techniques can be used to apply the amphiphile-modified sorbent to filter fibers or other substrate supports. For example, the amphiphile-modified sorbent can be added to the filter fibers before they are formed into a filter cartridge, e.g., a tip for a cigarette. The amphiphile-modified sorbent can be added to the filter fibers, for example, in the form of a dry powder or a slurry. If the amphiphile-modified sorbent is applied in the form of a slurry, the fibers are allowed to dry before they are formed into a filter cartridge.

In another preferred embodiment, the amphiphile-modified sorbent is employed in a hollow portion of a cigarette filter. For example, some cigarette filters have a plug/space/plug configuration in which the plugs comprise a fibrous filter material and the space is simply a void between the two filter plugs. That void can be filled with the amphiphile-modified sorbent. An example of this embodiment is shown in FIG. 3. The amphiphile-modified sorbent can be in granular form or can be loaded onto a suitable support such as a fiber or thread.

In another embodiment, the amphiphile-modified sorbent is employed in a filter portion of a cigarette for use with a smoking device as described in U.S. Pat. No. 5,692,525, the entire content of which is hereby incorporated by reference. FIG. 8 illustrates one type of construction of a cigarette 100 which can be used with an electrical smoking device. As shown, the cigarette 100 includes a tobacco rod 60 and a filter portion 62 joined by tipping paper 64. The filter portion 62 preferably contains a tubular free-flow filter element 102 and a mouthpiece filter plug 104. The free-flow filter ele-

## 11

ment 102 and mouthpiece filter plug 104 may be joined together as a combined plug 110 with plug wrap 112. The tobacco rod 60 can have various forms incorporating one or more of the following items: an overwrap 71, another tubular free-flow filter element 74, a cylindrical tobacco plug 80 preferably wrapped in a plug wrap 84, a tobacco web 66 comprising a base web 68 and tobacco flavor material 70, and a void space 91. The free-flow filter element 74 provides structural definition and support at the tipped end 72 of the tobacco rod 60. At the free end 78 of the tobacco rod 60, the tobacco web 66 together with overwrap 71 are wrapped about cylindrical tobacco plug 80. Various modifications can be made to a filter arrangement for such a cigarette incorporating the amphiphile-modified sorbent.

In such a cigarette, amphiphile-modified sorbent can be incorporated in various ways such as by being loaded onto paper or other substrate material which is fitted into the passageway of the tubular free-flow filter element 102 therein. It may also be deployed as a liner or a plug in the interior of the tubular free-flow filter element 102. Alternatively, the amphiphile-modified sorbent can be incorporated into the fibrous wall portions of the tubular free-flow filter element 102 itself. For instance, the tubular free-flow filter element or sleeve 102 can be made of suitable materials such as polypropylene or cellulose acetate fibers and the amphiphile-modified sorbent can be mixed with such fibers prior to or as part of the sleeve forming process.

In another embodiment, the amphiphile-modified sorbent can be incorporated into the mouthpiece filter plug 104 instead of in the element 102. However, as in the previously described embodiments, amphiphile-modified sorbent may be incorporated into more than one constituent of a filter portion such as by being incorporated into the mouthpiece filter plug 104 and into the tubular free-flow filter element 102.

The filter portion 62 of FIG. 8 can also be modified to create a void space into which the amphiphile-modified sorbent can be inserted.

As explained above, amphiphile-modified sorbent can be incorporated in various support materials. When the amphiphile-modified sorbent is used in filter paper, the particles may have an average particle diameter of up to 100  $\mu\text{m}$ , preferably 2 to 50  $\mu\text{m}$ . When the amphiphile-modified sorbent is used in filter fibers or other mechanical supports, larger particles may be used. Such particles preferably have a mesh size from 20 to 60, and more preferably from 35 to 60 mesh.

The amount of amphiphile-modified sorbent employed in the cigarette filter by way of incorporation on a suitable support such as filter paper and/or filter fibers depends on the amount of constituents in the tobacco smoke and the amount of constituents desired to be removed. As an example, the filter paper and the filter fibers may contain, from 10% to 50% by weight of the amphiphile-modified sorbent.

Another embodiment relates to methods of making a filter. The methods comprise incorporating an amphiphile-modified sorbent having at least one amphiphilic compound bound to an inorganic molecular sieve substrate into a cigarette filter.

Most filters contain four main constituents: filter tow, plasticizer, plug wrap and adhesive. Often the filter tow comprises a bundle of cellulose acetate fibers or papers that are bound together using the plasticizer, which acts as a hardening agent. The filter is contained in the plug wrap, usually a paper wrapper, which is secured using an adhesive.

## 12

Any conventional or modified method of making cigarette filters may be used to incorporate the amphiphile-modified sorbent.

Another embodiment relates to methods of making cigarettes. In one embodiment, the method comprises: (i) providing a cut filler to a cigarette making machine to form a tobacco column; (ii) placing a paper wrapper around the tobacco column to form a tobacco rod; and (iii) attaching a cigarette filter incorporating an amphiphile-modified sorbent to the tobacco rod to form the cigarette.

Examples of suitable types of tobacco materials which may be used include flue-cured, Burley, Maryland or Oriental tobaccos, the rare or specialty tobaccos, and blends thereof. The tobacco material can be provided in, the form of tobacco lamination; processed tobacco materials such as volume expanded or puffed tobacco, processed tobacco stems such as cut-rolled or cut-puffed stems, reconstituted tobacco materials; or blends thereof. Tobacco substitutes may also be used.

In cigarette manufacture, the tobacco is normally employed in the forth of cut filler, i.e., in the form of shreds or strands cut into widths ranging from about  $1/10$  inch to about  $1/20$  inch or even  $1/40$  inch. The lengths of the strands range from between about 0.25 inches to about 3.0 inches. The cigarettes may further comprise one or more flavorants or other additives (e.g., burn additives, combustion modifying agents, coloring agents, binders, etc.) known in the art.

Cigarettes can be manufactured to any desired specification using standard or modified cigarette making techniques and equipment. The cigarettes may range from about 50 mm to about 120 mm in length. Generally, a regular cigarette is about 70 mm long, a "King Size" is about 85 mm long, a "Super King Size" is about 100 mm long, and a "Long" is usually about 120 mm in length. The circumference is from about 15 mm to about 30 mm in circumference, and preferably around 25 mm. The packing density is typically between the range of about 100  $\text{mg/cm}^3$  to about 300  $\text{mg/cm}^3$ , and preferably 150  $\text{mg/cm}^3$  to about 275  $\text{mg/cm}^3$ .

Yet another embodiment relates to methods of smoking the cigarette described above, which involve lighting the cigarette to form smoke and drawing the smoke through the cigarette, wherein during the smoking of the cigarette, the amphiphile-modified sorbent is capable of selectively adsorbing one or more selected constituents from mainstream smoke. Preferably at least 10%, 20%, 30%, 40%, 50% or more of the selected constituent is removed from the tobacco smoke by the sorbent.

"Smoking" of a cigarette means the heating or combustion of the cigarette to form smoke, which can be drawn in through the cigarette. Generally, smoking of a cigarette involves lighting one end of the cigarette and drawing the smoke through the mouth end of the cigarette, while the tobacco contained therein undergoes a combustion reaction. However, the cigarette may also be smoked by other means. For example, the cigarette may be smoked by heating the cigarette and/or heating using an electrical heater, as described in commonly-assigned U.S. Pat. Nos. 6,026,820; 5,988,176; 5,915,387; 5,692,526; 5,692,525; 5,666,976; and 5,499,636, for example.

While the invention has been described in detail with reference to preferred embodiments thereof, it will be apparent to one skilled in the art that various changes can be made, and equivalents employed, without departing from the scope of the invention.

All of the above-mentioned references are herein incorporated by reference in their entirety to the same extent as

if each individual reference was specifically and individually indicated to be incorporated herein by reference in its entirety.

What is claimed is:

1. A smoking article comprising an amphiphile-modified sorbent having at least one amphiphilic compound selected from the group consisting of an imidazoline, an ethoxylated amine, and a quaternary phospholipid bound to an inorganic molecular sieve substrate.

2. The smoking article of claim 1, wherein: (a) the smoking article is selected from the group consisting of a cigarette, a pipe, a cigar and a non-traditional cigarette; (b) the amphiphile-modified sorbent is located in a filter; (c) the amphiphile-modified sorbent is capable of removing at least some of at least one selected constituent of mainstream smoke by molecular sieving, ion exchange, hydrophobic interactions, chelation, chemical binding, or combinations thereof; (d) the amphiphile-modified sorbent selectively removes at least some of at least one selected constituent of mainstream smoke; (e) the amphiphile-modified sorbent is capable of removing at least some of a hydrocarbon compound constituent of mainstream smoke or a polar organic compound constituent of mainstream smoke; (f) the amphiphile-modified sorbent is capable of removing at least some of an organic compound constituent of mainstream smoke; (g) the amphiphile-modified sorbent is capable of removing at least one selected constituent of mainstream smoke selected from the group consisting of aldehyde, carbon monoxide, 1,3-butadiene, isoprene, acrolein, acrylonitrile, hydrogen cyanide, o-toluidine, 2-naphthylamine, nitrogen oxide, benzene, N-nitrosonornicotine, phenol, catechol, benz(a)anthracene, and benzo(a)pyrene; (h) the amphiphile-modified sorbent is capable of removing at least some of an aldehyde constituent of mainstream smoke; (i) the amphiphilic compound comprises from about 4 to about 24 carbon; or (j) the amphiphilic compound comprises from about 6 to about 18 carbons.

3. The smoking article of claim 2, wherein the smoking article is a cigarette.

4. The smoking article of claim 2, wherein the filter is a mono filter, a dual filter, a triple filter, a cavity filter, a recessed filter or a free-flow filter.

5. The smoking article of claim 1, wherein: (a) the inorganic molecular sieve substrate is selected from the group consisting of zeolite, aluminophosphate, silicate, aluminosilicates, and mixtures thereof; (b) the inorganic molecular sieve substrate is a zeolite selected from the group consisting of zeolite ZSM-5, zeolite A, zeolite X, zeolite Y, zeolite K-G, zeolite ZK-5, zeolite Beta, zeolite ZK-4, and mixtures thereof; (c) the amphiphilic compound is covalently bound to the surface of the inorganic molecular sieve substrate; (d) the amphiphile-modified sorbent is in particle form having an average mesh size from about 20 mesh to about 60 mesh; (f) the smoking article is a cigarette including from about 50 mg to about 300 mg of the amphiphile-modified sorbent; (g) the smoking article is a cigarette including from about 100 mg to about 200 mg of the amphiphile-modified sorbent; or (h) the molecular sieve comprises a mesoporous molecular sieve.

6. A cigarette filter comprising an amphiphile-modified sorbent having at least one amphiphilic compound, selected from the group consisting of an imidazoline, an ethoxylated amine, and a quaternary phospholipid bound to an inorganic molecular sieve substrate.

7. The cigarette filter of claim 6, wherein: (a) the amphiphile-modified sorbent is capable of removing at least some of at least one selected constituent of mainstream smoke by molecular sieving, ion exchange, hydrophobic interactions, chelation, chemical binding, or combinations thereof; (b) the amphiphile-modified sorbent selectively removes at least some of at least one selected constituent of mainstream smoke; (c) the amphiphile-modified sorbent is capable of removing at least some of a hydrocarbon compound constituent of mainstream smoke, or a polar organic compound constituent of mainstream smoke; (d) the amphiphile-modified sorbent is capable of removing at least some of an organic compound constituent of mainstream smoke; (e) the amphiphile-modified sorbent is capable of removing at least one selected constituent of mainstream smoke selected from the group consisting of aldehyde, carbon monoxide, 1,3-butadiene, isoprene, acrolein, acrylonitrile, hydrogen cyanide, o-toluidine, 2-naphthylamine, nitrogen oxide, benzene, N-nitrosonornicotine, phenol, catechol, benz(a)anthracene, and benzo(a)pyrene; (f) the amphiphile-modified sorbent is capable of removing at least some of an aldehyde constituent of mainstream smoke; (g) the amphiphilic compound comprises from about 4 to about 24 carbons; or (h) the amphiphilic compound comprises from about 6 to about 18 carbons.

8. The cigarette filter of claim 6, wherein: (a) the inorganic molecular sieve substrate is selected from the group consisting of zeolite, aluminophosphate, silicate, aluminosilicates, and mixtures thereof; (b) the inorganic molecular sieve substrate is a zeolite selected from the group consisting of zeolite ZSM-5, zeolite A, zeolite X, zeolite Y, zeolite K-G, zeolite ZK-5, zeolite Beta, zeolite ZK-4, and mixtures thereof; (c) the amphiphilic compound is covalently bound to the surface of the inorganic molecular sieve substrate; (d) the amphiphilic compound is electrostatically bound to the surface of the inorganic molecular sieve substrate; or (e) the amphiphile-modified sorbent is in particle form having an average mesh size from about 20 mesh to about 60 mesh.

9. The cigarette filter of claim 6, wherein: (a) the smoking article is a cigarette including from about 50 mg to about 300 mg of the amphiphile-modified sorbent; (b) the smoking article is a cigarette including from about 100 mg to about 200 mg of the amphiphile-modified sorbent; (c) the filter is selected from the group consisting of a mono filter, a dual filter, a triple filter, a cavity filter, a recessed filter, and a free-flow filter; (d) the filter comprises at least one material selected from the group consisting of cellulose acetate tow, cellulose paper, mono cellulose, mono acetate, and combinations thereof; (e) the amphiphile-modified sorbent is incorporated into one or more cigarette filter parts selected from the group consisting of shaped paper insert, a plug, a space, cigarette filter paper, and a free-flow sleeve; (f) the amphiphile-modified sorbent is incorporated with cellulose acetate fibers forming a plug or a free-flow filter element; (g) the amphiphile-modified sorbent is incorporated with polypropylene fibers forming a plug or free-flow filter element; (h) the amphiphile-modified sorbent is incorporated in at least one of a mouthpiece filter plug, a first tubular filter element adjacent to the mouthpiece filter plug, and a second tubular filter element adjacent to the first tubular element; or (i) the amphiphile-modified sorbent is incorporated in at least one part of a three-piece filter including a mouthpiece filter plug, a first filter plug adjacent to the mouthpiece filter plug, and a second filter plug adjacent to the first filter plug.

10. A method of making a cigarette filter, the method comprising incorporating an amphiphile-modified sorbent having at least one amphiphilic compound, selected from the

**15**

group consisting of an imidazoline, an ethoxylated amine and a quaternary phospholipid bound to an inorganic molecular sieve substrate into a cigarette filter.

**11.** The method of claim **10**, wherein the filter is a mono filter, a dual filter, a triple filter, a cavity filter, a recessed filter or a free-flow filter.

**12.** A method of making a cigarette, the method comprising:

- (i) providing a cut filler to a cigarette making machine to form a tobacco column;
- (ii) placing a paper wrapper around the tobacco column to form a tobacco rod;
- (iii) providing a cigarette filter comprising an amphiphile-modified sorbent having at least one amphiphilic compound, selected from the group consisting of an imidazoline, an ethoxylated amine and a quaternary phospholipid bound to an inorganic molecular sieve substrate; and
- (iv) attaching the cigarette filter to the tobacco rod to form the cigarette.

**16**

**13.** A method of smoking a cigarette comprising an amphiphile-modified sorbent having at least one amphiphilic compound, selected from the group consisting of an imidazoline, an ethoxylated amine and a quaternary phospholipid comprising lighting the cigarette to form smoke and drawing the smoke through the cigarette, wherein during the smoking of the cigarette, the amphiphile-modified sorbent removes at least one selected constituent from mainstream smoke.

**14.** The method of claim **13**, wherein at least one selected constituent of mainstream smoke is removed by molecular sieving, ion exchange, hydrophobic interactions, chelation, chemical binding, or combinations thereof.

**15.** The method of claim **13**, wherein the amphiphile-modified sorbent selectively removes at least some of an organic compound constituent of mainstream smoke.

**16.** The method according to claim **13**, wherein the amphiphile-modified sorbent removes at least some of an aldehyde constituent of mainstream smoke.

\* \* \* \* \*